# EUROPEAN PATENT SPECIFICATION

(11) **EP 0 629 511 B1**
(45) Date of publication and mention of the grant of the patent: **01.12.1999**
(21) Application number: 94303938.8
(22) Date of filing: 01.06.1994
(51) Int. Cl.: B41M 5/165, B41M 5/145, B41M 5/30, B41M 5/28

(54) **Recording material**
Aufzeichnungsmaterial
Matériau d'enregistrement

(30) Priority: 01.06.1993 JP 15613293
(43) Date of publication of application: 21.12.1994
(73) Proprietor: FUJI PHOTO FILM CO., LTD., Kanagawa 250-01 (JP)
(72) Inventor: Sano, Shojiro, c/o Fuji Film Co., Ltd., Fujinomya-shi, Shizouka (JP)
(74) Representative: Arthur, Bryan Edward

(56) References cited:
- EP-A- 0 176 161
- EP-A- 0 520 639
- GB-A- 2 210 701
- GB-A- 2 220 909
- JP-A- 50 090 409
- US-A- 4 583 104

## Description

### FIELD OF THE INVENTION

The present invention relates to a recording material which is employable for a pressure sensitive material and a heat sensitive material.

### BACKGROUND OF THE INVENTION

Recording materials that contain both a microcapsule containing an electron-donating color former (hereinafter may be referred to as *"*color former*"*) dissolved in a solvent and an electron-accepting developer (hereinafter may be referred to as *"*developer*"*), are widely used. In the recording material, the color former reacts with the developer to form a colored image.

Such recording material is roughly divided into a pressure sensitive material and a heat sensitive material. The pressure sensitive material utilizes the mechanisms that the microcapsule containing the color former is ruptured by application of pressure to form a color image through the reaction of the color former with the developer. The pressure sensitive recording material includes a no-carbon-paper-type recording material that a color former layer comprising a microcapsule containing a color former (hereinafter may be referred to as *"*color former layer*"*) and a developer layer containing an electron-accepting developer (hereinafter may be referred to as "developer layer") are respectively formed on surfaces of separate supports or separate surfaces of one support and are in contact with each other to be used; and a self-coloring-type pressure sensitive recording material (e.g., pressing-type paper or self-contained paper) comprising a self-coloring layer having both the color former and the developer provided on one side surface of a support.

The no-carbon-paper-type recording material consists of a upper paper having a color former layer provided on one side surface of a support (which usually is paper sheet), an intermediate paper having a color former layer provided on one side surface of a support and a developer layer on another side surface of the support, and a lower paper having a developer layer provided on one side surface of a support. The intermediate paper is usually used in the form of two or more sheets. Such no-carbon-paper-type recording material is employed by bringing the color former into contact with the developer to form a colored image.

In the self-coloring-type pressure sensitive recording material, when pressure is applied to a surface having a self-coloring layer, a microcapsule in the layer is ruptured to form a color image on the self-coloring layer through the reaction of the color former with the developer. Therefore, the material is usually employed for writing or drawing an image such as a letter on a paper placed on the self-coloring layer with writing instruments or a typewriter, for directly printing a colored image on the self-coloring layer with a printer or a typewriter, or for printing a letter for OCR (optical character reader) on the self-coloring layer.

In preparation of plural copies, a self-coloring-type pressure sensitive recording material using a upper paper having a self-coloring layer provided on one side surface of a support and a color former layer on another side surface of the support, in combination with an intermediate paper having a color former layer and developer layer and a lower paper having a developer layer is occasionally employed. Types of the self-coloring layer of the self-coloring-type pressure sensitive recording material includes a two layers-type layer consisting of a color former layer containing a microcapsule containing a color former and a developer layer containing a developer which are superposed upon each other, and a one layer-type layer consisting of one layer containing a color former and a developer.

The heat sensitive recording materials containing a microcapsule, for example, are those having a heat sensitive layer which contains a microcapsule containing a color former and a developer, as described in Japanese Patent Provisional Publications No. 63(1988)-265682 and No. 1(1989)-105782. Such recording material has the advantages that can be designed for OHP (over head projector) or multicolor type.

The microcapsule, which is contained in the above recording materials, contains a color former dissolved in a solvent. It is necessary that such solvent is capable of dissolving the color former. Examples of the solvents generally include kerosine, paraffin, naphthene oil, alkylated biphenyl, alkylated terphenyl, chlorinated paraffin, alkylated napthalene, diaryl alkane and phthalic acid ester. However, such solvents generally give off ill smell. Some of them are harmful to living things so that they have the danger that bring out enivornment pollution (e.g., poor working condition). In more detail, when the recording material is prepared using such solvents or the recording material containing the solvents is used, the above problem occur.

A method for the manufacture of microcapsules usable in pressure sensitive recording sheets is described in GB-A-2220909.

A heat sensitive recording material composed of an electron donating colorless dye and an electron accepting compound is known from US 4583104.

Japanese Patent Provisional Publication No. 50(1975)-90409 describes a process for preparation of a pressure sensitive recording paper comprising the steps of dissolving a color former in an animal or vegetable oil heated at 105 to 260°C to prepare a color former solution, and forming a microcapsule layer containing the color former solution on support.

The animal or vegetable oils used in the process are natural edible materials mainly composed of triglyceride. Such oils have no ill smell and assured safety from the viewpoint of ecology, and further are available at low prices. Therefore, the oils are suitable for a solvent for the color former solution contained in the microcapsule.

However, the animal or vegetable oils generally do not have a sufficient dissolving power required for dissolving a color former and therefore it is difficult to increase a concentration of the color former in its solution. In the process described in the Japanese Patent Provisional Publication No. 50(1975)-90409, a color former is dissolved in an animal or vegetable oil by heating the oil at a high temperature of 105 to 260°C. However, such heating brings about deterioration of quality of the oil due to oxidation, and the heated oil occasionally gives off ill smell. Further, the oil itself inhibits occasionally coloring of the color former (i.e., desensitizes the color former).

### SUMMARY OF THE INVENTION

It is an object of the present invention to provide a recording material which has no ill smell and assured safety, and shows coloring of high density.

It is another object of the invention to provide a pressure sensitive recording material which has no ill smell and assured safety, and shows coloring of high density.

It is a further object of the invention to provide a heat sensitive recording material which has no ill smell and assured safety, and shows coloring of high density.

The present inventor has studied to find a color former that easily dissolves in glycerides such as vegetable oils in high concentration at relatively low temperature. In more detail, finding of such color former enables the glycerides to use as a solvent for the color former solution contained in the microcapsule.

As a result, he has found the specific fluoran compound of the following formula (I) as such color former. Thus, he has been able to complete the invention.

The invention resides in a recording material which comprises a support, microcapsules containing an electron-donating color former dissolved in a solvent and an electron-accepting developer, the color former and the developer being provided on the support;

characterised in that the solvent comprises a glyceride and the electron-donating color former comprises a fluoran compound of the formula (I): in which R¹ represents an alkyl group of 1 to 4 carbon atoms, R² represents a branched alkyl group of 4 to 12 carbon atoms or a tetrahydrofurfuryl group, and each of R³ and R⁴ represents independently a hydrogen atom, a halogen atom or a methyl group, provided that R¹ differs from R², the fluoran compound of the formula (I) being contained in the glyceride in an amount of 3 to 8% by weight based on the amount of the glyceride with the proviso that the glyceride is not an animal oil.

Preferred embodiments of the recording material are as follows:
(1) The recording material wherein R¹ represents methyl, ethyl, n-propyl or isopropyl, R² represents isobutyl, sec-butyl, isopentyl, isohexyl, 2-methylhexyl, 2-ethylhexyl, 2-ethyldecyl and tetrahydrofurfuryl, and each of R³ and R⁴ represents independently hydrogen, chlorine or methyl, there being no case that R¹ and R² represent the same group.
(2) The recording material wherein the solvent is vegetable oil.
(3) The recording material described above (2) wherein the vegetable oil.is at least one selected from the group consisting of soybean oil, sesame oil, corn oil, rapeseed oil, cotton seed oil, olive oil, peanut oil, castor oil, palm oil, coconut oil, sunflower oil, camellia oil, palm kernel oil, hardened oil and epoxidated oil.
(4) The recording material wherein the solvent consists essentially of triglyceride.
(5) The recording material wherein the microcapsule is prepared by dissolving the electron-donating color former in the glyceride at a temperature of 80 to 100°C and encapsulating the obtained solution.
(6) The recording material wherein the developer comprises clay materials.

Further, the invention resides in a pressure sensitive recording material comprising a support, a pressure rupturable color former layer comprising microcapsules which contains an electron-donating color former dissolved in a solvent and a developer layer comprising an electron-accepting developer;
wherein the solvent comprises a glyceride with the proviso that the glyceride is not an animal oil and the electron-donating color former comprises a fluoran compound of the above formula (I).

Furthermore, the invention resides in a pressure sensitive recording material which comprises a upper paper comprising a paper sheet and a pressure rupturable color former layer provided on the paper sheet, and a lower paper comprising a paper sheet and a developer layer provided on the paper sheet, said color former layer comprising a microcapsule which contains an electron-donating color former dissolved in a solvent and said developer layer comprising an electron-accepting developer;
wherein the solvent comprises a glyceride and the electron-donating color former comprises a fluoran compound of the formula (I).

Preferred embodiment of the above pressure sensitive recording material are as follows:
(1) The pressure sensitive recording material which further has at least one intermediate paper which has a paper sheet, a color former layer provided on one side surface of the paper sheet and a developer layer on another side surface of the paper sheet between the upper paper and the lower paper.

The recording material of the invention employs glycerides according to claim 1 as a solvent for dissolving the color former. The glycerides generally give off no ill smell and are not harmful to living things. Therefore, they do not bring out poor working condition, and naturally do not environmental pollution. Further, the recording material shows coloring of high density due to use of the specific fluoran compound (color former) in combination with the glycerides because the fluoran compound is not desensitized by the glycerides. Hence, the recording material of the invention is one that has assured safety and shows coloring of high density. Particularly, it is useful for a pressure sensitive recording material.

### BRIEF DESCRIPTION OF DRAWINGS

Fig. 1 is a schematic sectional view of a typical structure of the no-carbon-paper-type pressure sensitive recording material according to the invention.
Fig. 2 is a schematic sectional view of a typical structure of the self-coloring-type pressure sensitive recording material according to the invention.
Fig. 3 is a schematic sectional view of another structure of the self-coloring-type pressure sensitive recording material according to the invention.

### DETAILED DESCRIPTION OF THE INVENTION

The recording material of the invention contains both a microcapsule containing an electron-donating color former dissolved in a solvent and an electron-accepting developer. The recording material is not restricted in its form so long as it contains a microcapsule containing a color former comprising a fluoran compound of the formula (I) dissolved in a glyceride with the proviso that the glyceride is not animal oil.

The typical structures of the recording materials of the invention are described below.
Fig. 1 shows a typical structure of the no-carbon-paper-type pressure sensitive recording material. A upper paper 1 has a color former layer 3 provided on one side surface of a support 2. An intermediate paper 4 has a developer layer 5 provided on one side surface of a support 6 and a color former layer 7 on another side surface of the support 6. A lower paper 8 has a developer layer 9 provided on one side surface of a support 10. The three paper are superposed in the order as shown in Fig. 1. Although the intermediate paper 4 is usually used in the form of a pile of two or more sheets, it may be not used. Recording (formation of image) is generally performed by applying pressure to the opposite surface of the color former layer 3 of the support 2 to bring the color former into contact with the developer.
Fig. 2 shows a typical structure of the self-coloring-type pressure sensitive recording material. Both a color former layer 11 and a developer layer 12 are provided on one side surface of a support 13.
Fig. 3 shows another structure of the self-coloring-type pressure sensitive recording material. A self-coloring layer 14 containing both a color former and a developer is provided on one side surface of a support 13.

The heat sensitive recording material has the same structure as that shown in Fig. 3. The self-coloring layer 14 corresponds to a heat sensitive layer.

The recording material of the invention is characterized by the use of and the amount used of the specific compound as the color former contained in the microcapsule and glyceride as the solvent for dissolving the color former, as defined in claim 1. As for an example of the no-carbon-paper-type pressure sensitive material, a detail explanation is given below. It will be easily understand that the similar effect is obtained in recording materials having other forms.

Glyceride employed in the invention is used for dissolving the color former. Any natural glycerides and synthesis glycerides are employable in the invention. Further, any of triglycerides, diglycerides, monoglycerides and a mixture thereof are employable in the invention. It is preferred that the glyceride is mainly composed of triglyceride. The glyceride preferably is a ester of glycerin and saturated fatty acid.

Examples of the glycerides include 1-monocaprin, 1-monoundecanoin, 1-monolaurin, 1-monotridecanoin, 1-monomyristin, 1-monopentadecanoin, 1-monopalmitin, 1-monostearin, 1-monoolein, 1-monoelaidin, 1-monolinolenin, 1-monoarachin, 1-monobutyrin, 2-monocaprin, 2-monolaurin, 2-monomyristin, 2-monopalmitin, 2-monostearin,
1,3-dicaprin, 1,3-diundecanoin, 1,3-dilaurin, 1,3-ditridecanoin, 1,3-myristin, 1,3-pentadecanoin, 1,3-dipalmitin, 1,3-distearin, 1,3-diarachin, 1,2-dilaurin, 1,2-dimyristin, 1,2-dipalmitin, 1,2-distearin,
triacetin, tributyrin, 1-aceto-2,3-dipalmitin, 1-aceto-2,3-distearin, tricaproin, 1-caproyl-2,3-distearin, 1-caproyl-2,3-diolein, tricaprylin, 1-elaido-2,3-dicaprylin, 1-linoleo-2,3-dicaprylin, 1-caprylyl-2,3-distearin, 1-caprylyl-2,3-diolein, trinonanoin, tricaprin, 1-lauro-2,3-dicaprin, 1-myristo-2,3-dicaprin, 1-palmito-2,3-dicaprin, 1-stearo-2,3-dicaprin, 1-oleo-2,3-dicaprin, 1-elaido-2,3-dicaprin, 1-linoleo-2,3-dicaprin, 2-lauro-1,3-dicaprin, 1-capryl-2,3-dilaurin, 1-capryl-2-lauro-3-myristin, 2-myristo-1,3-dicaprin, 1-capryl-2,3-dimylistin, 2-palmito-1,3-dicaprin, 1-capryl-2,3-dipalmitin, 2-stearo-1,3-dicaprin, 1-capryl-2,3-distearin, 2-oleo-1,3-dicaprin, 1-capryl-2,3-diolein, 1-capryl-2,3-dielaidin, 1-capryl-2,3-dilaurin, trilaurin, 1-myristo-2,3-dilaurin, 1-palmito-2,3-dilaurin, 1-stearo-2,3-dilaurin, 1-oleo-2,3-dilaurin, 1-elaido-2,3-dilaurin, 1-linoleo-2,3-dilaurin, 2-myristo-1,3-dilaurin, 1-lauro-2,3-dimyristin, 1-lauro-2-myristo-3 palmitin, 2-palmito-1,3-dilaurin, 1-lauro-2,3-dipalmitin, 2-stearo-1,3-dilaurin, 1-lauro-2,3-distearin, 2-oleo-1,3-dilaurin, 1-lauro-2,3-diolein, 1-lauro-2,3-dielaidin, 1-lauro-2,3-dilinolein, 2-capryl-1,3-dimyristin, 1-myristo-2-capryl-3-stearin, trimyristin, 1-palmito-2,3-dimyristin, 1-stearo-2,3-dimyristin, 1-oleo-2,3-dimyristin, 1-elaidino-2,3-dimyristin, 1-linoleo-2,3-dimyristin, 2-palmito-1,3-dimyrstin, 1-myristo-2,3-dipalmitin, 1-myristo-2-palmito-3-stearin, 2-stearo-1,3-dimyristin, 1-myristo-2,3-distearin, 2-oleo-1,3-dimyristin, 1-myristo-2,3-diolein, 1-myristo-2,3-dielaidin, 1-mylisto-2,3-dilinolein, 2-capryl-1,3-dipalmitin, 1-palmito-2-capryl-3-stearin, 2-lauro-1,3-dipalmitin, 1-palmito-2-lauro-3-stearin, 2-myristo-1,3-dipalmitin, tripalmitin, 1-stearo-2,3-dipalmitin, 1-oleo-2,3-dipalmitin, 1-linoleo-2,3-dipalmitin, 2-stearo-1,3-dipalmitin, 1-palmito-2,3-distearin, 2-oleo-1,3-dipalmitin, 1-palmito-2,3-diolein, 1-palmito-2,3-dilinolein, 2-capryl-1,3-stearin, 2-lauro-1,3-distearin, 2-myristo-1,3-distearin, 2-palmito-1,3-distearin, tristearin, 1-oleo-2,3-distearin, 1-linoleo-2,3-distearin, 2-oleo-1,3-distearin, 1-stearo-2,3-diolein, 1-stearo-2,3-dilinolein, 2-stearo-1,3-diolein and a mixture thereof.

Although these glycerides may be synthesis glycerides or natural oil, it is convenience to use the natural oil. Preferred examples of the natural oil include vegetable oils such as soybean oil, sesame oil, corn oil, rapeseed oil, cotton seed oil, olive oil, peanut oil, castor oil, palm oil, coconut oil, sunflower oil, camellia oil and palm kernel oil. These oils are employable singly or in combination. Further, hardened oil prepared by hydrogenation of unsaturated glyceride and epoxidated oil prepared by epoxidation of unsaturated bond of unsaturated glyceride are also employable as glyceride of the invention.

In the invention, a conventional solvent mentioned previously is employable in an amount of not more than 30 weight % per glyceride), in combination with the glyceride.

The color former employed in the invention is a fluoran compound of the formula (I) mentioned previously. Examples of the alkyl group of 1 to 4 carbon atoms represented by R¹ include methyl, ethyl, n-propyl, isopropyl, n-butyl, sec-butyl and tert-butyl. Preferred are methyl, ethyl, n-propyl and isopropyl. Particularly, ethyl is preferred.

Examples of the branched alkyl group of 4 to 12 carbon atoms represented by R² include isobutyl, sec-butyl, tert-butyl, isopentyl, sec-pentyl, tert-pentyl, isohexyl, 2-methylhexyl, 2-ethylhexyl and 2-ethyldecyl. Preferred examples of the group represented by R² include isobutyl, sec-butyl, isopentyl, isohexyl, 2-methylhexyl, 2-ethylhexyl, 2-ethyldecyl and tetrahydrofurfuryl. Particularly, isobutyl and tetrahydrofurfuryl are preferred.

Preferred examples of the group represented by R³ include hydrogen, chlorine and methyl. Particularly, methyl is preferred.

Preferred examples of the group represented by R⁴ include hydrogen, chlorine and methyl. Particularly, hydrogen is preferred.

Preferred examples of the fluoran compound of the formula (I) include 2-anilino-3-methyl-6-N-ethyl-N-isobutylaminofluoran, 2-anilino-3-methyl-6-N-ethyl-N-isopentylaminofluoran, 2-anilino-3-methyl-6-N-methyl-N-isobutylaminofluoran, 2-anilino-3-methyl-6-N-methyl-N-isopentylaminofluoran, 2-anilino-3-methyl-6-N-ethyl-N-isohexylaminofluoran, 2-anilino-3-methyl-6-N-ethyl-N-(2-ethylhexyl)aminofluoran, 2-toluidino-3-methyl-6-N-ethyl-N-isobutylaminofluoran, 2-anilino-3-methyl-6-Nethyl-N-(2-ethyldecyl)aminofluoran, 2-anilino-3-methyl-6-N-n-propyl-N-isobutylaminofluoran, 2-anilino-3-methyl-6-N-isopropyl-N-isobutylaminofluoran, 2-(o-chloroanilino)-6-N-ethyl-N-isobutylaminofluoran, 2-anilino-3-chloro-6-N-ethyl-N-(sec-butyl)aminofluoran, 2-anilino-3-methyl-6-N-ethyl-N-tetrahydrofurfurylaminofluoran and 2-anilino-3-methyl-6-N-methyl-N-tetrahydrofurfurylaminofluoran.

In the invention, known color formers can be employed together with the fluoran compound for purpose of controlling tone. Examples of the known color formers include triphenylmethanphthalide compounds, fluoran compounds other than the fluoran compounds of formula (I), phenothiazine compounds, indolylphthalide compounds, leucoauramine compounds, rhodaminelactam compounds, triphenylmethan compounds, triazene compounds and spiropyran compounds. The fluoran compound of formula (I) is preferably used in the amount of not less than 70 weight % based on the total amount of the used color formers to give an image of high coloring density.

The microcapsule containing the color former of the fluoran compound having the formula (I) is prepared by dissolving the color former in the solvent of the glyceride. The fluoran compound is preferably dissolved in a solvent of the glyceride at a temperature of 80 to 100°C. In the case of a temperature lower than 80°C, the fluoran compound is not easily dissolved in the glyceride. In the case of a temperature higher than 100°C, the glyceride is occasionally deteriorated. The fluoran compound of the formula (I) is contained in the solution of the color former in the amount of 3 to 8 % by weight based on the amount of the glyceride. Color formers other than the fluoran compound of the formula (I) are dissolved in the glyceride at the temperature within the above range so long as in the amount of lower than 1 weight %. For dissolving these color formers in the above amount (3 to 8 weight %), it is required to heat a mixture containing them to approx. 150°C.

The microcapsule used in the invention and containing the color former dissolved in the solvent is prepared according to the known method such as an interfacial polymerization method, an internal polymerization method, a phase separation method, an external polymerization method or a coacervation method.

As the shell material of the microcapsule, water-insoluble or oil-insoluble polymers which is used in the conventional pressure sensitive material are employable. The shell material is preferred to be polyurethane/polyurea resin having high resistance to heat-fogging. The microcapsule dispersion for forming the shell of polyurethane/polyurea resin to incorporate the color former, is prepared by, for example, the steps of dissolving a multi-functional isocyanate compound and a multi-functional hydroxyl compound (further UV absorbent if desired) in the solution prepared by dissolving the color former in glyceride as above, dispersing the resultant solution to a hydrophilic liquid, adding a multi-functional amine to the resultant dispersing solution, and coating the polyurethane/polyurea resin around a drop of the glyceride solution. The multi-functional hydroxyl compound and the multi-functional amine may be used in combination as above, or either of them may be used.

The dispersing solution of the microcapsule prepared above is directly employed as a coating solution for forming the color former layer. Otherwise, the coating solution is prepared by adding further a binder and/or an agent for protecting a capsule to the dispersing solution. The resultant coating solution is coated on the support according to a known coating method and the coated layer is dried. Thus, the color former layer for the no-carbon-paper-type pressure sensitive recording material is formed. Examples of the binder include a water-soluble binder and a latex binder and examples of the agent for protecting a capsule include powders of cellulose, powders of starch and talc.

As materials of the support, materials employed for the support of the conventional pressure sensitive recording material and the conventional heat sensitive recording material. Examples of the materials of the support include a paper made of pulp, a surface treated paper, a synthetic paper made of plastic and a plastic film.

The coated amount of the color former layer formed on the support after drying generally is in the range of 0.05 to 0.30 g/m², and preferably is in the range of 0.08 to 0.20 g/m².

Examples of the developer contained in the developer layer of the no-carbon-paper-type pressure sensitive recording material include clay materials such as acid clay, activated clay, attapulgite, zeolite, bentonite and kaolin, metal salts of aromatic carboxylic acids (e.g., salicylic acid derivatives), and a phenol formaldehyde resin. The developer preferably is clay materials from the viewpoint of ecology.

A coating solution for forming the above developer layer is prepared according a known method. For example, the coating solution may further contain a binder. Examples of the binder include natural or synthetic polymers such as styrene/butadiene copolymer latex, polyvinyl acetate latex, polyacrylate latex, polyvinyl alcohol, polyacrylic acid, maleic anhydride/styrene copolymer, starch, casein, carboxymethyl cellulose and methyl cellulose. The developer layer is formed on the support utilizing a known coating method.

The coated amount of the developer layer formed on the support after drying generally is in the range of 0.1 to 4.0 g/m², and preferably is in the range of 0.2 to 3.0 g/m².

The no-carbon-paper-type pressure sensitive recording material according to the invention has a composition similar to a conventional one except for employing the fluoran compound of the formula (I) as color former and the glyceride as the solvent for dissolving the color former. Therefore, the no-carbon-paper-type pressure sensitive material of the invention can be prepared utilizing the known process.

As for other recording materials such as the self-coloring-type pressure sensitive recording material and the heat sensitive recording material described previously, they have a composition similar to conventional one except for employing the above specific compounds as color former in the amount mentioned in claim 1 and for employing a glyceride as defined in claim 1 as the solvent for dissolving the color former which are contained in the microcapsule. Therefore, the recording materials can be prepared utilizing the known processes.

The present invention is further described by the following examples.

### EXAMPLE 1

### (Preparation of coating solution for forming color former layer)

In 120 g of cotton seed oil, 5.0 g of 2-anilino-3-methyl-6-N-ethyl-N-isobutylaminofluoran as a color former was dissolved by heating at 90°C for 1 hour. In the resultant oily solution, 10 g of a carbodiimide-modified diphenylmethandiisocyanate (Milionate MTL, (Trade Mark) available from Nippon Polyurethane Co., Ltd.) and 5 g of a biuret body of hexamethylenediisocyanate (Sumijule N-3200 (Trade Mark); available from Sumitomo Bayer Urethane Co., Ltd.) as a multi-functional isocyanate compound, and 3.0 g of butylene oxide adduct of ethylenediamine (adduct molar number of butylene oxide to ethylenediamine: 16.8 moles; Molecular weight: 1,267) as an alkylene oxide adduct of amine were dissolved to prepare a primary solution.

Subsequently, 10 g of polyvinyl alcohol and 5 g of carboxymethylcellulose were dissolved in 140 g of water to prepare a secondary solution. The primary solution was poured into the secondary solution while the secondary solution was vigorously stirred. Thus oil-in-water emulsion was formed. When a size of the oil droplet of the emulsion became 5.0 µm, the stirring power was weakened and then 100 g of water of 20°C was added to the emulsion. Subsequently, the temperature of the emulsion was gradually raised to 70°C and this temperature was kept for 90 minutes. Thus a capsule solution was obtained.

To the obtained capsule solution, 80 g of a polyvinyl alcohol 15 weight % solution, 30 g (solid content) of carboxyl-modified SBR (styrene butadiene rubber) latex and 60 g of starch particles (mean particle size: 15 µm) were added, and further the solution was adjusted to 20 weight % by the addition of water to prepare a coating solution for forming a color former layer which contains a microcapsule containing a color former.

### (Preparation of color former sheet)

On the one side of a paper of 50 g/m², the above coating solution for forming a color former layer was so coated as to have 4.0 g/m² in terms of solid content using an air-knife coater, and dried to prepare the color former sheet. This color former sheet scarcely gave off smell.

### (Preparation of coating solution "A" for forming developer layer)

A mixture of 200 g of activated clay, 20 g of sodium carbonate, 8 g of magnesium oxide, 1 g of sodium hexametaphosphate, 20 g of 20 weight % sodium hydroxide and 500 g of water was dispersed by means of a cady mill. To the resultant dispersing solution, 40 g (solid content) of a carboxyl-modified SBR (styrene butylene rubber) latex and 60 g of a starch aqueous solution (10 weight %) were added to prepare the coating solution *"*A*"* for forming a developer layer.

### (Preparation of developer sheet "A")

On the one side of a paper of 50 g/m², the above coating solution *"*A*"* for forming a developer layer was so coated as to have 6.0 g/m² in terms of solid content using an air-knife coater, and dried to prepare the developer sheet *"*A*"*.

### (Evaluation of developed color density)

The resultant color former sheet was placed on the resultant developer sheet *"*A*"* in such a manner that the color former layer and the developer layer came into contact each other. Load of 300 kg/cm² was applied to the resultant composite to form a developed image on the developer layer. After the image of the developer layer was allowed to stand at room temperature for 24 hours, its density (D) was measured using Macbeth reflective densitometer. The result is set forth in Table 1.

### EXAMPLE 2

### (Preparation of color former sheet)

Procedures of Example 1 was repeated except for using the same amount of soybean oil instead of cotton seed oil to prepare the coating solution for forming a color former layer and then to prepare the color forming sheet. The resultant color former sheet scarcely gave off smell.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### EXAMPLE 3

### (Preparation of color former sheet)

Procedures of Example 1 was repeated except for using the same amount of corn oil instead of cotton seed oil to prepare the coating solution for forming a color former layer and then to prepare the color forming sheet. The resultant color former sheet scarcely gave off smell.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### EXAMPLE 4

### (Preparation of color former sheet)

Procedures of Example 1 was repeated except for using the same amount of epoxidated soybean oil instead of cotton seed oil to prepare the coating solution for forming a color former layer and then to prepare the color forming sheet. The resultant color former sheet scarcely gave off smell.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### EXAMPLE 5

### (Preparation of color former sheet)

Procedures of Example 1 was repeated except for using the same amount of 1,2-dilaurin instead of cotton seed oil to prepare the coating solution for forming a color former layer and then to prepare the color forming sheet. The resultant color former sheet scarcely gave off smell.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### COMPARISON EXAMPLE 1

### (Preparation of color former sheet)

Procedures of Example 1 was repeated except for using the same amount of 1-phenyl-1-xylylethane instead of cotton seed oil to prepare the coating solution for forming a color former layer and then to prepare the color forming sheet. The resultant color former sheet gave off a stimulative smell.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### COMPARISON EXAMPLE 2

### (Preparation of color former sheet)

5.0 g of 2-anilino-3-methyl-6-N,N-diethylaminofluoran as a color former was dissolved in 120 g of cotton seed oil by heating at 90°C for 1 hour. However, most of the color former was not dissolved in the oil and therefore the insoluble color former formed the deposit in the solution of the oil and the color former.

Procedures of Example 1 was repeated except for using the oily solution prepared above instead of one of Example 1, to prepare the coating solution for forming a color former layer and then to prepare the color forming sheet.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### COMPARISON EXAMPLE 3

### (Preparation of color former sheet)

5.0 g of 2-anilino-3-methyl-6-N-ethyl-N-cyclohexylaminofluoran as a color former was dissolved in 120 g of cotton seed oil by heating at 90°C for 1 hour. However, most of the color former was not dissolved in the oil and therefore the insoluble color former formed the deposit in the solution of the oil and the color former.

Procedures of Example 1 was repeated except for using the oily solution prepared above instead of one of Example 1, to prepare the coating solution for forming a color former layer and then to prepare the color forming sheet.

### (Evaluation of developed color density)

Using the resultant color former sheet and the developer sheet *"*A*"* prepared in the same manner as Example 1, the evaluation of the developed color density was performed in the same manner as Example 1. The result is set forth in Table 1.

### EXAMPLE 6

### (Preparation of coating solution for forming color former layer)

In 100 g of rapeseed oil, 2.5 g of 2-anilino-3-methyl-6-N-ethyl-N-tetrahydrofurfurylaminofluoran and 2.5 g of 2-anilino-3-methyl-6-N-ethyl-N-isopentylaminofluoran as a color former was dissolved by heating at 95°C for 30 minutes. To the resultant oily solution, 20 g of paraffin solvent (IP solvent 1620, available from Idemitsu protochemical Co., Ltd.) was added to prepare a color former oily solution.

12 g of acid-treated gelatin having an isoelectric point of 8.2 and 10 g of gum Arabic were dissolved in 80 g of water (40°C). To the solution, 0.2 g of Turkey red oil (that is, sulphonated castor oil) was added as an emulsifier to prepare a colloidal solution. The above color former oily solution was added to the colloidal solution with vigorously stirring to emulsify, and thus an oil in water emulsion was obtained. With stirring, 370 g of warm water (40°C) was added to the emulsion and 20% hydrochloric acid was dropwise added to the emulsion to adjust its pH to 4.4. A vessel having the emulsion therein was cooled from the outside with stirring the emulsion to set a colloid wall deposited on the oil drop to gel. When the temperature of the emulsion became 10°C with continuously stirring, 3.0 g of formaldehyde 37 % solution was added to the emulsion and further 40 g of 7 weight % aqueous solution of sodium salt of carboxymethylcellulose (etherification degree: 0.75) was added. Then, sodium hydroxide 10 weight % aqueous solution was dropwise added to the emulsion till the pH became 10, and the vessel having the emulsion therein was heated from the outside to raise its temperature to 40°C. The emulsion was kept at this temperature for 1 hour to prepare a capsule solution containing the color former.

To the resultant capsule solution, 120 g of oxidized starch 15 % aqueous solution and 40 g of starch particle having mean particle size of 12 µm were added. Further, water was added to the capsule solution to adjust its solid content (concentration) to 20 weight %. Thus, the coating solution for forming a color former layer which contains the microcapsule containing the color former was prepared.

### (Preparation of color former sheet)

On the one side of a paper of 50 g/m², the above coating solution for forming the color former layer was so coated as to have 4.5 g/m² in terms of solid content using an air-knife coater, and was dried to prepare the color former sheet. This color former sheet scarcely gave off smell.

### (Preparation of coating solution "B" for forming developer layer)

A mixture of 120 g of calcium carbonate, 20 g of zinc oxide, 5 g of zinc 3,5-bis(α-methylbenzyl)salicylate, 1 g of sodium hexametaphosphate and 200 g of water was subjected to atomization treatment using a sand mill to prepare a dispersing solution. To 300 g of the dispersing solution, 200 g of 9 % aqueous solution of polyvinyl alcohol (PVA-117, available from Kuraray Co., Ltd.) and 4 g (solid content) of a carboxyl-modified SBR (styrene butylene rubber) latex (SN307, available from Sumitomo Norgatack Co., Ltd.) were added and adjusted the solid content to 20 weight % by addition of water to prepare the coating solution *"*B*"* for forming a developer layer.

### (Preparation of developer sheet "B")

On the one side of a paper of 50 g/m², the above coating solution *"*B*"* for forming a developer layer was so coated as to have 4.5 g/m² in terms of solid content using an air-knife coater, and dried to prepare the developer sheet *"*B*"*.

### (Evaluation of developed color density)

The obtained color former sheet was placed on the resultant developer sheet *"*B*"* in such a manner that the color former layer and the developer layer came into contact. Using the resultant composite, the evaluation of the developed color density was performed in the same manner as that of Example 1. The result is set forth in Table 1.

### COMPARISON EXAMPLE 4

### (Preparation of color former sheet)

Procedures of Example 6 was repeated except for using the same amount of monoisopropylbiphenyl instead of rapeseed oil to prepare the coating solution for forming a color former layer and then to prepare the color forming sheet. The resultant color former sheet gave off a stimulative smell.

### (Evaluation of developed color density)

Using the resultant color former sheet and the developer sheet *"*B*"* prepared in the same manner as Example 6, the evaluation of the developed color density was performed in the same manner as Example 1. The result is set forth in Table 1.

### COMPARISON EXAMPLE 5

### (Preparation of color former sheet)

In 120 g of cotton seed oil, 2.5 g of 2-anilino-3-methyl-6-N,N-dibutylaminofluoran and 2.5 g of 2-anilino-3-methyl-6-N,N-diethylaminofluoran as a color former was dissolved by heating at 90°C for 1 hour. However, most of the color formers were not dissolved in the oil and therefore the insoluble color former formed the deposit in the solution of the oil and the color former.

Although a capsule was tried to form using the oily solution of the oil and the color former prepared above in the same manner as procedures of Example 6, aggregation of the oily drops was generated with violence in the course of formation of the capsule. Therefore, the capsule was not formed and thus the color forming sheet which contains capsule containing the color former was not prepared.

**Table 1**

| | Color density (D) |
|---|---|
| Example 1 | 0.76 |
| Example 2 | 0.75 |
| Example 3 | 0.75 |
| Example 4 | 0.77 |
| Example 5 | 0.75 |
| Comp. Ex. 1 | 0.75 |
| Comp. Ex. 2 | 0.33 |
| Comp. Ex. 3 | 0.40 |
| Example 6 | 0.72 |
| Comp. Ex. 4 | 0.71 |

Any recording materials prepared in the Examples scarcely gave off smell. Further, these materials showed the color images of high color densities with combination of the developer sheets. In contrast, the recording materials of Comparison Examples 1 and 4 which used materials other than glyceride as a solvent, gave off a stimulative smell to give unpleasant feeling to users, although they showed the color images of high color densities similar to those of Examples. Further, in the recording materials of Comparison Examples 2, 3 and 5 which used glyceride as a solvent and the color formers outside of the scope of the invention, the color formers were little dissolved or were insoluble in the triglyceride and therefore the use of them did not result in formation of capsule, or merely resulted in formation of capsule which gave the color image of an extremely low density on the developer sheet.

The color formers used in Comparison Examples 2 and 3 have structure similar to the fluoran compounds of formula (I) of the invention, but it was unexpected that the color formers showed an extreme low color density compared with those used in the invention.

## Claims

1. A recording material which comprises a support, microcapsules containing an electron-donating color former dissolved in a solvent and an electron-accepting developer, the color former and the developer being provided on the support;
characterised in that the solvent comprises a glyceride and the electron-donating color former comprises a fluoran compound of the formula (I): in which R¹ represents an alkyl group of 1 to 4 carbon atoms, R² represents a branched alkyl group of 4 to 12 carbon atoms or a tetrahydrofurfuryl group, and each of R³ and R⁴ represents independently a hydrogen atom, a halogen atom or a methyl group, provided that R¹ differs from R², the fluoran compound of the formula (I) being dissolved in the glyceride in an amount of 3 to 8% by weight based on the amount of the glyceride with the proviso that the glyceride is not an animal oil.

2. The recording material as defined in Claim 1, characterised in that R¹ represents methyl, ethyl, n-propyl or isopropyl, R² represents isobutyl, sec-butyl, isopentyl, isohexyl, 2-methylhexyl, 2-ethylhexyl, 2-ethydecyl and tetrahydrofurfuryl, and each of R³ and R⁴ represents independently hydrogen, chlorine or methyl.

3. The recording material as defined in Claim 1 or Claim 2, characterised in that the solvent is a vegetable oil, a hardened oil or an epoxidated oil.

4. The recording material as defined in Claim 3, characterised in that the vegetable oil is at least one oil selected from the group consisting of soybean oil, sesame oil, corn oil, rapeseed oil, cotton seed oil, olive oil, peanut oil, castor oil, palm oil, coconut oil, sunflower oil, camellia oil and palm kernel oil.

5. The recording material as defined in any preceding claim, characterised in that the solvent consists essentially of a triglyceride.

6. The recording material according to any preceding claim, characterised in that the microcapsules are obtainable by dissolving the electron-donating color former in the glyceride at a temperature of 80 to 100°C and encapsulating the obtained solution.

7. The recording material as defined in any preceding claim, characterised in that the developer comprises clay materials.

8. A pressure sensitive recording material which has both a color former layer comprising pressure rupturable microcapsules which contain an electron-donating color former dissolved in a solvent and a developer layer comprising an electron-accepting developer;
characterised in that the solvent comprises a glyceride and the electron-donating color former comprises a fluoran compound of the formula (I) as defined in claim 1, the fluoran compound of the formula (I) being contained in the glyceride in an amount of 3 to 8% by weight based on the amount of glyceride with the proviso that the glyceride is not an animal oil.

9. The pressure sensitive recording material as defined in Claim 8, characterised in that R¹ represents methyl, ethyl, n-propyl or isopropyl, R² represents isobutyl, sec-butyl, isopentyl, isohexyl, 2-methylhexyl, 2-ethylhexyl, 2-ethyldecyl and tetrahydrofurfuryl, and each of R³ and R⁴ represents independently hydrogen, chlorine or methyl.

10. The pressure sensitive recording material as defined in Claim 8 or Claim 9, characterised in that the solvent is a vegetable oil, hardened oil or an epoxidated oil.

11. The pressure sensitive recording material as defined in Claim 10, characterised in that the vegetable oil is at least one selected from the group consisting of soybean oil, sesame oil, corn oil, rapeseed oil, cotton seed oil, olive oil, peanut oil, castor oil, palm oil, coconut oil, sunflower oil, camellia oil and palm kernel oil.

12. The pressure sensitive recording material as defined in any one of Claims 8 to 11, characterised in that the solvent consists essentially of a triglyceride.

13. The pressure sensitive recording material as defined in any one of Claims 8 to 12, characterised in that the microcapsule is obtainable by dissolving the electron-donating color former in the glyceride at a temperature of 80 to 100°C and encapsulating the obtained solution.

14. The pressure sensitive recording material as defined in any one of Claims 8 to 13, characterised in that the developer comprises clay materials.

15. A pressure sensitive recording material which comprises an upper paper comprising a paper sheet with a color former layer provided on the paper sheet, and a lower paper comprising a paper sheet with a developer layer provided on the paper sheet, said color former layer comprising pressure rupturable microcapsules which contain an electron-donating color former dissolved in a solvent and said developer layer comprising an electron-accepting developer;
characterised in that the solvent comprises a glyceride and the electron-donating color former comprises a fluoran compound of the formula (I) defined in claim 1, the fluoran compound of the formula (I) being contained in the glyceride in an amount of 3 to 8% by weight based on the amount of the glyceride with the proviso that the glyceride is not an animal oil.

16. The pressure sensitive recording material as defined in Claim 15, characterised in that the material further comprises at least one intermediate paper which has a paper sheet, a color former layer provided on one side surface of the paper sheet and a developer layer on another side surface of the paper sheet between the upper paper and the lower paper.

17. The recording material as defined in any preceding claim, wherein the solvent comprises the glyceride and a solvent selected from the group of kerosine, paraffin, naphthene oil, alkylated biphenyl, alkylated terphenyl, chlorinated paraffin, alkylated naphthalene, diaryl alkane and phthalic acid ester in an amount of not more than 30 weight % of the glyceride.

## Patentansprüche

1. Ein Aufzeichnungsmaterial, das einen Träger, Mikrokapseln enthaltend einen Elektronen abgebenden Farbbildner gelöst in einem Lösungsmittel und einen Elektronen aufnehmenden Entwickler enthält, wobei der Farbbildner und der Entwickler auf dem Träger vorgesehen sind;
dadurch gekennzeichnet, daß das Lösungsmittel ein Glycerid enthält und der Elektronen abgebende Farbbildner eine Fluoranverbindung der Formel (I) enthält: in welcher R¹ einer Alkylgruppe mit 1 bis 4 Kohlenstoffatomen entspricht, R² einer verzweigten Alkylgruppe mit 4 bis 12 Kohlenstoffatomen oder einer Tetrahydrofurfurylgruppe entspricht, und jedes der R³ und R⁴ unabhängig voneinander einem Wasserstoffatom, einem Halogenatom oder einer Methylgruppe entspricht, unter der Bedingung bzw. Voraussetzung (provided that), daß R¹ von R² verschieden ist, wobei die Fluoranverbindung der Formel (I) in dem Glycerid in einer Menge von bis 8 Gew.-% bezogen auf die Menge an Glycerid gelöst ist, unter der Bedingung, daß das Glycerid kein tierisches Öl ist.

2. Das Aufzeichnungsmaterial gemäß Anspruch 1, dadurch gekennzeichnet, daß R¹ Methyl, Ethyl, n-Propyl oder Isopropyl entspricht, R² Isobutyl, sec-Butyl, Isopentyl, Isohexyl, 2-Methylhexyl, 2-Ethylhexyl, 2-Ethyldecyl (2-ethydecyl) und Tetrahydrofurfuryl entspricht und jedes der R³ und R⁴ unabhängig voneinander Wasserstoff, Chlor oder Methyl entspricht.

3. Das Aufzeichnungsmaterial gemäß Anspruch 1 oder Anspruch 2, dadurch gekennzeichnet, daß das Lösungsmittel ein pflanzliches Öl, ein gehärtetes Öl oder ein epoxidiertes Öl ist.

4. Das Aufzeichnungsmaterial gemäß Anspruch 3, dadurch gekennzeichnet, daß das pflanzliche Öl mindestens ein Öl ist, ausgewählt aus der Gruppe bestehend aus Sojabohnenöl, Sesamöl, Maisöl (corn oil), Rapssamenöl, Baumwollsamenöl, Olivenöl, Erdnußöl, Rizinusöl, Palmöl, Kokosnußöl, Sonnenblumenöl, Kamelienöl und Palmkernöl.

5. Das Aufzeichnungsmaterial gemäß irgendeinem der vorangehenden Ansprüche, dadurch gekennzeichnet, daß das Lösungsmittel im wesentlichen aus einem Triglycerid besteht.

6. Das Aufzeichnungsmaterial gemäß irgendeinem der vorangehenden Ansprüche, dadurch gekennzeichnet, daß die Mikrokapseln erhältlich sind durch Lösen des Elektronen abgebenden Farbbildners in dem Glycerid bei einer Temperatur von 80 bis 100°C und Einschließen der erhaltenen Lösung.

7. Das Aufzeichnungsmaterial gemäß irgendeinem der vorangehenden Ansprüche, dadurch gekennzeichnet, daß der Entwickler Ton- bzw. Lehmmaterialien (clay materials) enthält.

8. Ein druckempfindliches Aufzeichnungsmaterial, das sowohl eine Farbbildnerschicht hat, die drucksprengbare Mikrokapseln enthält, die einen Elektronen abgebenden Farbbildner gelöst in einem Lösungsmittel enthalten, als auch eine Entwicklerschicht, die einen Elektronen aufnehmenden Entwickler enthält:
dadurch gekennzeichnet, daß das Lösungsmittel ein Glycerid enthält und der Elektronen abgebende Farbbildner eine Fluoranverbindung der Formel (I) gemäß Anspruch 1 enthält, wobei die Fluoranverbindung der Formel (I) in dem Glycerid in einer Menge von 3 bis 8 Gew.-% bezogen auf die Menge des Glycerids enthalten ist, unter der Voraussetzung, daß das Glycerid kein tierisches Öl ist.

9. Das druckempfindliche Aufzeichnungsmaterial gemäß Anspruch 8, dadurch gekennzeichnet, daß R¹ Methyl, Ethyl, n-Propyl oder Isopropyl entspricht, R² Isobutyl, sec-Butyl, Isopentyl, Isohexyl, 2-Methylhexyl, 2-Ethylhexyl, 2-Ethyldecyl und Tetrahydrofurfuryl entspricht, und jedes der R³ und R⁴ unabhängig voneinander Wasserstoff, Chlor oder Methyl entspricht.

10. Das druckempfindliche Aufzeichnungsmaterial gemäß Anspruch 8 oder Anspruch 9, dadurch gekennzeichnet, daß das Lösungsmittel ein pflanzliches Öl, ein gehärtetes Öl oder ein epoxidiertes Öl ist.

11. Das druckempfindliche Aufzeichnungsmaterial gemäß Anspruch 10, dadurch gekennzeichnet, daß das pflanzliche Öl mindestens eines ist, das aus der Gruppe ausgewählt ist, die besteht aus Sojabohnenöl, Sesamöl, Maisöl (corn oil), Rapssamenöl, Baumwollsamenöl, Olivenöl, Erdnußöl, Rizinusöl, Palmöl, Kokosnußöl, Sonnenblumenöl, Kameliennöl und Palmkernöl.

12. Das druckempfindliche Aufzeichnungsmaterial gemäß irgendeinem der Ansprüche 8 bis 11, dadurch gekennzeichnet, daß das Lösungsmittel im wesentlichen aus einem Triglycerid besteht.

13. Das druckempfindliche Aufzeichnungsmaterial gemäß irgendeinem der Ansprüche 8 bis 12, dadurch gekennzeichnet, daß die Mikrokapsel erhältlich ist durch Lösen des Elektronen abgebenden Farbbildners in dem Glycerid bei einer Temperatur von 80 bis 100°C und Einschließen der erhaltenen Lösung.

14. Das druckempfindliche Aufzeichnungsmaterial gemäß irgendeinem der Ansprüche 8 bis 13, dadurch gekennzeichnet, daß der Entwickler Ton- bzw. Lehmmaterialien enthält.

15. Ein druckempfindliches Aufzeichnungsmaterial, das ein oberes Papier enthält, das eine Papierfläche mit einer Farbbildnerschicht enthält, die auf der Papierfläche vorgesehen ist, und ein unteres Papier, das eine Papierfläche mit einer Entwicklerschicht enthält, die auf der Papierfläche vorgesehen ist, wobei die Farbbildnerschicht drucksprengbare Mikrokapseln enthält, die einen Elektronen abgebenden Farbbildner enthalten, der in einem Lösungsmittel gelöst ist und die Entwicklerschicht einen Elektronen aufnehmenden Entwickler enthält;
dadurch gekennzeichnet, daß das Lösungsmittel ein Glycerid enthält und der Elektronen abgebenden Farbbildner eine Fluoranverbindung der Formel (I) gemäß Anspruch 1 enthält, wobei die Fluoranverbindung der Formel (I) in dem Glycerid in einer Menge von 3 bis 8 Gew.-% bezogen auf die Menge des Glycerids enthalten ist, unter der Voraussetzung, daß das Glycerid kein tierisches Öl ist.

16. Das druckempfindliche Aufzeichnungsmaterial gemäß Anspruch 15, dadurch gekennzeichnet, daß das Material ferner wenigstens ein intermediäres Papier enthält, das eine Papierfläche hat, eine Farbbildnerschicht, die auf einer Seitenoberfläche der Papierfläche vorgesehen ist und eine Entwicklerschicht auf einer anderen Seitenoberfläche der Papierfläche zwischen dem oberen Papier und dem unteren Papier.

17. Das Aufzeichnungsmaterial gemäß irgendeinem der vorangehenden Ansprüche, worin das Lösungsmittel das Glycerid und ein Lösungsmittel enthält, das aus der Gruppe aus Kerosin, Paraffin, Naphthenöl, alkyliertem Biphenyl, alkyliertem Terphenyl, chloriertem Paraffin, alkyliertem Naphthalin, Diarylalkan und Pthalsäureester in einer Menge von nicht mehr als 30 Gew.-% des Glycerids ausgewählt ist.

## Revendications

1. Matériau d'enregistrement qui comprend un support, des microcapsules contenant un copulant chromogène donneur d'électrons dissous dans un solvant, et un révélateur accepteur d'électrons, le copulant chromogène et le révélateur étant fournis sur le support ;
caractérisé en ce que le solvant comprend un glycéride, et le copulant chromogène donneur d'électrons comprend un fluoranne de formule (I) : dans laquelle R¹ représente un groupe alkyle ayant de 1 à 4 atomes de carbone, R² représente un groupe alkyle ramifié ayant de 4 à 12 atomes de carbone ou un groupe tétrahydrofurfuryle, et chacun des radicaux R³ et R⁴ représente indépendamment de l'autre un atome d'hydrogène, un atome d'halogène ou un groupe méthyle, à la condition que R¹ soit différent de R², le fluoranne de formule (I) étant dissous dans le glycéride en une quantité de 3 à 8 % en poids par rapport à la quantité du glycéride, à la condition que le glycéride ne soit pas une huile d'origine animale.

2. Matériau d'enregistrement selon la revendication 1, caractérisé en ce que R¹ représente le groupe méthyle, éthyle, n-propyle ou isopropyle, R² représente le groupe isobutyle, sec-butyle, isopentyle, isohexyle, 2-méthylhexyle, 2-éthylhexyle, 2-éthyldécyle et tétrahydrofurfuryle, et chacun des radicaux R³ et R⁴ représente indépendamment de l'autre un atome d'hydrogène ou de chlore, ou le groupe méthyle.

3. Matériau d'enregistrement selon la revendication 1 ou 2, caractérisé en ce que le solvant est une huile végétale, une huile durcie ou une huile époxydée.

4. Matériau d'enregistrement selon la revendication 3, caractérisé en ce que l'huile végétale est au moins une huile choisie dans l'ensemble constitué de l'huile de soja, de l'huile de sésame, de l'huile de maïs, de l'huile de colza, de l'huile de graine de coton, de l'huile d'olive, de l'huile d'arachide, de l'huile de ricin, de l'huile de palme, de l'huile de copra, de l'huile de tournesol, de l'huile de camellia, et de l'huile de palmiste.

5. Matériau d'enregistrement selon l'une quelconque des revendications précédentes, caractérisé en ce que le solvant est essentiellement constitué d'un triglycéride.

6. Matériau d'enregistrement selon l'une quelconque des revendications précédentes, caractérisé en ce que l'on obtient les microcapsules en dissolvant le copulant chromogène donneur d'électrons dans le glycéride à une température de 80 à 100°C, et en encapsulant la solution obtenue.

7. Matériau d'enregistrement selon l'une quelconque des revendications précédentes, caractérisé en ce que le révélateur comprend des matériaux à base d'argile.

8. Matériau d'enregistrement sensible à la pression, qui possède tant une couche de copulant chromogène comprenant des microcapsules pouvant se rompre sous l'effet d'une pression, qui contiennent un copulant chromogène donneur d'électrons dissous dans un solvant, qu'une couche d'un révélateur comprenant un révélateur accepteur d'électrons,
caractérisé en ce que le solvant comprend un glycéride et le copulant chromogène donneur d'électrons comprend un fluoranne de formule (I) selon la revendication 1, le fluoranne de formule (I) étant contenu dans le glycéride en une quantité de 3 à 8 % en poids par rapport au poids du glycéride, à la condition que le glycéride ne soit pas une huile d'origine animale.

9. Matériau d'enregistrement sensible à la pression selon la revendication 8, caractérisé en ce que R¹ représente le groupe méthyle, éthyle, n-propyle ou isopropyle, R² représente le groupe isobutyle, sec-butyle, isopentyle, isohexyle, 2-méthylhexyle, 2-éthylhexyle, 2-éthyldécyle et tétrahydrofurfuryle, et chacun des radicaux R³ et R⁴ représente indépendamment de l'autre un atome d'hydrogène ou de chlore, ou le groupe méthyle.

10. Matériau d'enregistrement sensible à la pression selon la revendication 8 ou 9, caractérisé en ce que le solvant est une huile végétale, une huile durcie ou une huile époxydée.

11. Matériau d'enregistrement sensible à la pression selon la revendication 10, caractérisé en ce que l'huile végétale est au moins une huile choisie dans l'ensemble constitué de l'huile de soja, de l'huile de sésame, de l'huile de maïs, de l'huile de colza, de l'huile de graine de coton, de l'huile d'olive, de l'huile d'arachide, de l'huile de ricin, de l'huile de palme, de l'huile de copra, de l'huile de tournesol, de l'huile de camellia, et de l'huile de palmiste.

12. Matériau d'enregistrement sensible à la pression selon l'une quelconque des revendications 8 à 11, caractérisé en ce que le solvant est essentiellement constitué d'un triglycéride.

13. Matériau d'enregistrement sensible à la pression selon l'une quelconque des revendications 8 à 12, caractérisé en ce que l'on obtient les microcapsules en dissolvant le copulant chromogène donneur d'électron dans le glycéride a une température de 80 à 100°C, et en encapsulant la solution obtenue.

14. Matériau d'enregistrement sensible à la pression selon l'une quelconque des revendications 8 à 13, caractérisé en ce que le révélateur comprend des matériaux à base d'argile.

15. Matériau d'enregistrement sensible à la pression, qui comprend un papier supérieur, comprenant une feuille de papier comportant une couche d'un copulant chromogène disposée sur la feuille de papier, et un papier inférieur comprenant une feuille de papier avec une couche de révélateur disposée sur la feuille de papier, ladite couche de copulant chromogène comprenant des microcapsules pouvant se rompre sous l'effet d'une pression, qui contiennent un copulant chromogène donneur d'électrons dissous dans un solvant, et ladite couche de révélateur comprenant un accepteur d'électrons, caractérisé en ce que le solvant comprend un glycéride et le copulant chromogène donneur d'électrons comprend un fluoranne de formule (I) selon la revendication 1, le fluoranne de formule (I) étant contenu dans le glycéride en une quantité de 3 à 8 % en poids par rapport au poids du glycéride, à la condition que le glycéride ne soit pas une huile d'origine animale.

16. Matériau d'enregistrement sensible à la pression selon la revendication 15, caractérisé en ce que le matériau comprend en outre au moins un papier intermédiaire qui possède une feuille de papier, une couche de copulant chromogène disposée sur une face de la feuille de papier et une couche de révélateur sur l'autre face de la feuille de papier, entre le papier supérieur et le papier inférieur.

17. Matériau d'enregistrement selon l'une quelconque des revendications précédentes, dans lequel le solvant comprend le glycéride et un solvant choisi dans l'ensemble comprenant le kérosène, la paraffine, les huiles naphthéniques, le biphényle alkylé, le terphényle alkylé, la paraffine chlorée, le napthalène alkylé, les diarylalcanes et des phtalates, en une quantité non supérieure à 30 % en poids du glycéride.
